# EUROPEAN PATENT SPECIFICATION

(11) **EP 1 769 097 B1**
(45) Date of publication and mention of the grant of the patent: **26.03.2008**
(21) Application number: 05767835.1
(22) Date of filing: 26.07.2005
(51) Int. Cl.: C22C 38/00, C22C 38/12, C22C 38/26

(54) **SHAPED STEEL EXCELLENT IN FIRE RESISTANCE AND PRODUCING METHOD THEREFOR**
FORMSTAHL MIT HOHER HITZEBESTÄNDIGKEIT UND FORMSTAHLHERSTELLUNGSVERFAHREN
ACIER PROFILE PRESENTANT D'EXCELLENTES CARACTERISTIQUES DE RESISTANCE AU FEU ET PROCEDE DE PRODUCTION ASSOCIE

(30) Priority: 28.07.2004 JP 2004220454; 28.07.2004 JP 2004220337; 15.07.2005 JP 2005207185
(43) Date of publication of application: 04.04.2007
(73) Proprietor: Nippon Steel Corporation, Tokyo 100-8071 (JP)
(72) Inventor: YOSHIDA, Suguru, c/o NIPPON STEEL CORPORATION, Futtsu-shi, Chiba 293-8511 (JP); EDA, Kazuhiko, c/o NIPPON STEEL CORPORATION, Sakai-shi, Osaka 590-8540 (JP); KITA, Hiroshi, c/o NIPPON STEEL CORPORATION, Sakai-shi, Osaka 590-8540 (JP)
(74) Representative: Vossius & Partner
(86) International application number: PCT/JP2005/013999
(87) International publication number: WO 2006/011618

(56) References cited:
- EP-A- 0 347 156
- EP-A- 0 589 424
- EP-A- 1 026 275
- EP-A- 1 182 268
- EP-A- 1 277 848
- US-A1- 2003 063 996
- DATABASE COMPENDEX [Online] ENGINEERING INFORMATION, INC., NEW YORK, NY, US; UEDA SYUZO ET AL: "RELATION BETWEEN PRECIPITATION BEHAVIOR OF Mo, V AND Nb AND YIELD STRENGTH IN NORMALIZED AND TEMPERED STEEL" XP002345283 Database accession no. EIX79050000050 -& TETSU TO HAGANE DEC 1978, vol. 64, no. 14, December 1978 (1978-12), pages 2177-2186, XP009053939
- GOPE N ET AL: "INFLUENCE OF LONG-TERM AGING AND SUPERIMPOSED CREEP STRESS ON THE MICROSTRUCTURE OF 0.50CR-0-50MO-0.25V STEEL" METALLURGICAL TRANSACTIONS A. PHYSICAL METALLURGY AND MATERIALS SCIENCE, METALLURGICAL SOCIETY OF AIME. NEW YORK, US, vol. 23A, no. 8, August 1992 (1992-08), pages 2193-2204, XP001007362
- LEE W B ET AL: "Influence of Mo on precipitation hardening in hot rolled HSLA steels containing Nb" SCRIPTA MATERIALIA, ELSEVIER, NEW YORK, NY, US, vol. 43, no. 4, 28 July 2000 (2000-07-28), pages 319-324, XP004326136 ISSN: 1359-6462

## Description

The present invention relates to a novel shaped steel, such as H-shaped steel, I-shaped steel, angle steel, channel steel, etc., which is used as a building construction material, with a low yield ratio and having excellence in toughness and fire resistance, and a method for producing the same.

The legislation about "new code to design fire-resistant structures" was enacted on March, 1987 in Japan. After that, fire-resistant steel materials, which secure high strength at high temperature without or with less fire-resistant wrapping, have been desired.

As for shaped steels, according to the trend, a lot of technologies for securing fire-resistance to steel were proposed. For example, it was proposed that strength, such as strength and yield ratio, at high temperature, such as 600°C, was secured by employing technologies of precipitation strengthening using Mo-based carbides.

For example, JP-A-9-104944 proposes a fire-resistant shaped steel using precipitation strengthening technology and oxide metallurgy technology. Oxide metallurgy technology is a technology, which can control the number of oxides, which oxides are obtained by deoxidization of the dissolved oxygen in steel using Ti, B and Mg. Oxide metallurgy technology provides the following effects.

In the production process of the shaped steel, different portions of the shaped steel are subjected respectively to different temperatures of finish-rolling and to different cooling rates resulting from the unevenness of the shape on the section of the steel, which causes lack of uniformity the microstructure of the section of the steel. This lack of uniformity of the microstructure, such as non-uniformity of grain size, leads to a lack of uniformity in the mechanical properties in the section of steel.

The flange portion, especially, the fillet part (see Fig.1), at which a flange portion and web portion meet, is less strained by rolling and forced to be processed at higher temperature compared with other portions.

In the section of a shaped steel (e.g., H-shaped steel), there can be a difference of around 150°C between the three portions of the fillet part, the 1/4 flange and the web (see FIG.1) in the temperature of finishing process. The different mechanical properties depending on portions caused by differences in the rolling temperature history of the portion should be eliminated.

The degree of finishing temperature dependency in the formation of microstructure during the hot rolling process can be reduced by dispersing the transformation nuclei, such as Ti oxide, in the ferrite grains and thereby expediting transformations in the grains. This leads to uniformity/homogenization of fine-grained microstructure, i.e., uniformity of mechanical properties. Furthermore, since the grain of the microstructure is not only homogenized but also finely grained, this leads to improved toughness.

The present inventors carried out extensive investigations in order to provide a shaped steel, such as H-shaped steel, which has a low yield ratio and is excellent in toughness and fire resistance and the method for producing the same. During extensive investigations, the inventors recognized the following possible technical issues.

At first, when the shaped steel excellent in fire-resistance is produced using oxide metallurgy technology, it is required for the processes, especially for casting the slab, billet, bloom, near net-shape slab, ingot, etc., to have complicated steps. Such complicated steps include oxygen content control before Ti is added and further Ti addition thereafter. Such steps may cause low productivity and high cost in the manufacture of the shaped steels.

Next, precipitation strengthening technology contributes to the fire-resistance of shaped steels, such as the strength and yield ratio at high temperature. However, in the case where Mo-based carbides, which contain mainly Mo₂C, are employed, such carbides may be solid-soluted in steel at the temperature range of 600 - 650°C if the components are within certain ranges. Consequently contribution to the strength of the steel provided by precipitation strengthening with alloy carbides and alloy carbonitrides may disappear.

The effect of precipitation strengthening depends on the amount of precipitates of alloy carbonitrides. Alloy carbonitrides include alloy carbides and alloy carbonitrides. Note that one or more metal may be present with the carbides or carbonitrides. Namely, here, alloy carbides mean metal carbides other than cementite. Hereinafter the amount of precipitate is expressed in mol fraction of precipitate and also may be simply referred to as "mol fraction of precipitate". The amount of precipitate depends upon the temperature. Further, such temperature dependence can be influenced by other factors, such as the carbon content of the steel and the thermodynamic characteristics based on the kinds of alloy carbides and alloy carbonitrides and so on.

As for the carbon content, if the content of C in the steel is sufficient in comparison with the contents of the metal elements, such as Mo, Ti, V, Nb, Cr, and capable of forming alloy carbonitrides, the amount of precipitate of alloy carbonitrides can be increased as the temperature decreases. This is because the content of C capable of forming precipitate increases as the carbon content solid-soluted (present in a solid-solution) in ferrite decreases when the temperature of the steel decreases.

Accordingly, the strength and yield ratio at the room temperature may be increased excessively even under the same thermal condition, such as the same temperature decrease, if the content of C is high and the mol fraction of precipitate of alloy carbides and alloy carbonitrides is increased excessively.
EP-A-0 347 156 discloses a process for manufacturing building construction steel having excellent fire resistance and low yield ratio which contains 0.005 to 0.10% of V as an optional element. EP-A-1 026 275 discloses a high-strength, high-toughness rolled shape steel contains 0.04 to 0.10% of V.

From such an analysis of technical issues, the inventors have recognized: i) it is preferred that the alloy carbides and alloy carbonitrides have not only thermodynamic stability, but also have the characteristic of being solid-soluted in the steel at the reheating temperature but not being solid-soluted at temperatures such as 600-650 °C, and ii) alloy carbides and alloy carbonitrides, which are capable of being soluted in the reheating process once and subsequently being precipitated in the cooling process of the hot rolling, can effectively contribute to precipitation strengthening.

The inventors, after close investigation, recognized that it is preferred to properly control the mol fraction of precipitate of alloy carbides and alloy carbonitrides at a high temperature range and at room temperature range, and that it is preferred to determine the components of the steel considering the following items.

(i) Suppressing the mol fraction of precipitate of alloy carbides and alloy carbonitrides in a room temperature range to prevent the strength and yield ratio at room temperature from being excessively increased; and (ii) attaining a specific mol fraction of precipitate of alloy carbides and alloy carbonitrides in order to obtain sufficient strength in a high temperature range.

Taking the above items into consideration, the inventors designed various alloy carbides and alloy carbonitrides and found that the amount of precipitate of alloy carbides and alloy carbonitrides can be controlled by making a proper balance in the amount (content) between the metal elements, such as Mo, Ti, V, Nb, Cr capable of forming alloy carbides and alloy carbonitrides, and C and N. It was found that the thermodynamic characteristics can be controlled by making a proper balance in the amount (content) between the metal elements.

More specifically, in the case where the Mo-based alloy carbide such as Mo₂C is the main constituent of the precipitate, which can be completely solid-soluted in steel at the temperature range of 600-650°C, contribution to the strength of the steel through precipitation strengthening by alloy carbides and alloy carbonitrides may disappear. However, it is found that the use of MCN type alloy carbonitrides, which are more stable than M₂C type alloy carbides in high temperature ranges, as a partial substitution for the Mo-based alloy carbides (i.e., an increase of precipitate amount of MCN type alloy carbonitrides in comparison with M₂C type alloy carbides, here "M" stands for metal other than ferrum) is very effective to solve the above issue.

That is, V replacing Mo partially therewith is added in order to form alloy carbonitrides other than Mo-based alloy carbides, and the generation of favorable alloy carbonitrides based mainly on V, Nb and Mo can be controlled by making a proper balance of the added amounts of V, Nb and Mo.

When referring to an expression such as "a room temperature", this is generally meant to refer to a temperature ranging from about 0°C to about 30°C. However, it is noted that the data at 300°C can be representative of the data at room temperature. This is because the amount of precipitate of alloy carbides and alloy carbonitrides increases very little between room temperature and 300°C. Rather, these precipitates of alloy carbides and alloy carbonitrides, measured in the present invention, occur mainly between 300°C and 600°C. This is due to the fact that as the temperature becomes closer to room temperature, the diffusion of solid solution elements such as metal elements, carbon and nitrogen, in the steel is extremely lowered in terms of precipitation behavior. More specifically, the equilibrium state of the precipitation remains almost unchanged between room temperature and 300°C. Thus, in the description of the present invention, the precipitation state at a temperature of 300°C can also be representative of that at room temperature. Further, the inventors have selected the temperature of 600°C as being a suitable "high temperature" for the measurement or evaluation of certain mechanical properties, as well as amounts of precipitate of alloy carbides and alloy carbonitrides. However, the "high temperature" is not limited to 600°C and can include other suitable temperatures.

An object of the invention is to provide a novel shaped steel, such as H-shaped steel, which is used as building construction material, with a low yield ratio and excellence in toughness and fire resistance, and the method for producing the same. The object may be accomplished by the following shaped steel and producing method thereof. The object above can be achieved by the features specified in the claims.

According to the present invention, a shaped steel, such as H-shaped steel having excellent strength at high temperature and excellent mechanical properties at room temperature can be obtained by forming alloy carbides and alloy carbonitrides containing mainly V and Mo in proper amounts by the specific process such as hot rolling a casted steel containing specific components. According to the present invention "casted steel" includes a slab, bloom, billet, near-net shape slab, ingot, etc.

FIG.1 shows locations where test pieces (specimen) are taken from an H-shaped steel 1. A first location is the center area of the flange 2 in the thickness direction (1/2 t₂) and one-fourth (1/4 B) position of the total flange width (B) away from the end of flange 2 in the flange width direction. A second location is the center area of the flange 2 in the thickness direction (1/2 t₂) and a half (1/2 B) position of the total flange width (B) in the flange width direction (fillet part 4). A third location is the center area of the web 3 in the thickness direction (1/2 t₁) and a half (1/2 H) position of the total web height (H) in the flange width direction.

FIG.2(a) is a graph showing a relationship between a total mol fraction of precipitate (which is a summation of M₂C type alloy carbides mol fraction and MCN type alloy carbonitrides mol fraction) and temperature, with respect to one example of the invention which contains V of 0. 35 %, where the M₂C type alloy carbides partially include V and Nb as a solid solution and the MCN type alloy carbonitrides include V and Nb as main components, and partially include Mo as a solid solution. The vertical axes of Figures 2 (a), 2 (b) and 3 are mol fraction of precipitates of alloy carbides, alloy carbonitrides and the total of alloy carbides and alloy carbonitrides.

FIG.2(b) is a graph showing the relationship between total mol fraction of precipitate and temperature, similar to FIG.2(a), where the V content is 0.22%.

FIG.3 is a graph showing relationships between temperature and each of the mol fractions of precipitates of M₂C type alloy carbides, MCN type alloy carbonitrides and a total of the M₂C type alloy carbides and the MCN type alloy carbonitrides using conventional technology. It is noted that a conventional method is any method in which neither the mol fraction of precipitate of alloy carbides and alloy carbonitrides at 600°C is 0,3% or more, nor the ratio of the mol fraction of precipitate of alloy carbides and alloy carbonitrides at 300°C to the mol fraction of precipitate of alloy carbides and alloy carbonitrides at 600°C is 2.0 or less.

The present invention is described more specifically below. Elements to be contained in the shaped steel of the present invention are described below. In this description, percent"%" represents "% by mass".

C is an element capable of improving the strength of steel. From the viewpoint of sufficient strength for structural steel, the content of C is 0. 03 % or more. C also has an influence on the toughness of the steel of the base material, the weld crack resistance and the toughness at heat affected zones (HAZ). From the viewpoint of such properties, the content of C is 0.15 % or less. Thus, the content of C is 0.03 to 0.15 %.

Si works as a deoxidizer (or oxygen scavenger) in the process of steel making and also influences the strength of the steel. From the viewpoint of sufficient strength for structural steel, the content of Si is 0.05 % or more. Si also influences the toughness at HAZ since excess amounts of Si may generate M-A (Martensite-Austenite) constituent of hardening structure, which may deteriorate the toughness at HAZ. In view of this, the content of Si is 0.5 % or less. Thus, the content of Si is 0.05 to 0.50 %.

Mn is an element capable of improving the strength and toughness of the mother phase. From this viewpoint, the content of Mn is 0.4 % or more. Mn also has an influence on the crack resistance and the toughness at HAZ. From the viewpoint of such properties, the content of Mn is 2. 0 % or less. Thus, the content of Mn is preferably 0.4 to 2.0 %.

Mo is an element, which is capable of forming Mo-based alloy carbide. In the present invention, it is thought that a shaped steel has excellent strength at room temperature and high temperature since the alloy carbide of Mo is precipitated. For sufficient strength of the shaped steel at high temperatures, the content of Mo is 0.1 % or more. Mo also improves the hardenability of steel. Excess content of Mo may deteriorate the toughness of steel and of HAZ since hardenability may be increased excessively. From the viewpoint of such properties, the content of Mo is 0.6 % or less. Thus, the content of Mo is 0.1 to 0.6 %, preferably 0.2 to 0.4 %, more preferably 0.2 to 0.3 %.

V is an element, which is capable of forming alloy carbonitride, and contributes to precipitation strengthening of steel. In the present invention, when V is used with Mo, V can be solid-soluted in the alloy carbide of M₂C, which contains Mo mainly, to form ((Mo, V)₂C), Further, V allows Mo to be solid-soluted in the alloy carbonitride of M(C, N), which contains V mainly, to form ((Mo,V) (C,N)) .

Properties of precipitate based on thermodynamics can be adjusted properly by transforming alloy carbides into either or both alloy carbides having the structure of M₂C and/or alloy carbonitrides having the structure of M (C, N) by adjusting the content of V and Mo. For conducting such transformation effectively, the content of V is 0.04 % or more.

When excess amounts of V are added, the amount of alloy carbonitrides may be increased excessively and the toughness of steel and of HAZ may be deteriorated. Therefore the content of V is 0.35 % or less.

On the other hand, in order to secure sufficient strength of fire resistance of a shaped steel at 600°C, for example, it is preferable to have a sufficient amount of the alloy carbonitride precipitated in the steel. For this purpose, the content of V is more than 0.20 %. Thus, the content of V is more than 0.20 to 0.35 %.

The precipitation of V-based alloy carbides having a structure of M₂C has been mainly controlled in order to obtain fire-resistance. However, it is more preferred that forming alloy carbonitrides having a structure of M(C, N) is mainly controlled in order to effectively improve the fire-resistance: From this viewpoint, the content of V is more than 0.20 %.

N is an element, which is capable of forming alloy carbonitrides. For obtaining sufficient precipitate, the content of N is 0. 002 % or more. Further, the content N is 0.012 % or less since excess amounts of N may cause deterioration of the toughness of steel. Thus, the content of N is 0.002 to 0.012 %.

A1 works as a strong deoxidizer (oxygen scavenger) in the process of steel making. However, A1 may form A1N combining with N, which leads to reduction in the amount of alloy carbonitrides (precipitate). Therefore, the A1 content is preferably 0.01 % or less.

Further, in the present invention, other optional components can be added.

Nb is an element, similar to V and Ti, which is capable of forming alloy carbonitrides, such as M(C,N), and contributing to precipitation strengthening. However, when the content of Nb is more than 0.06 %, it may not further improve the strength of the steel of the present invention by precipitation strengthening since the amount of alloy carbonitride which is not soluted at 1100-1300 °C, the temperature of heating, prior to hot rolling increases.

From the viewpoint of improvement of strength by the precipitation of alloy carbonitrides, the Nb content is preferably 0. 02 % or more. Thus, the content of Nb is preferably 0.02 to 0.06 %.

Ti is an element similar to Nb and V, which is capable of forming alloy carbonitrides such as M(C,N) and contributing to precipitation strengthening. In the present invention, Ti is solid-soluted in alloy carbonitride such as M(C,N), which is formed by adding V or a combination of V and Nb, to form alloy carbonitrides such as (V,Ti)(C,N) or (V,Ti,Nb) (C N). Accordingly, Ti influences the stability of alloy carbonitrides at high temperatures.

More specifically, alloy carbonitrides such as M(C,N) can extend the thermal stability range to higher temperatures when Ti is present. However, when the content of Ti exceeds 0.02 %, it may not contribute to precipitation strengthening since an amount of alloy carbonitride, which does not become solid-soluted at the heating temperature applied prior to hot rolling, such as 1100 - 1300°C, increases. Therefore, the content of Ti is preferably 0.02 % or less.

Cr is an element capable of not only improving the strength at room temperature and high temperature by increasing hardenability of steel and precipitation hardening, but is also capable of preventing the grain boundary from being oxidized (intergranular oxidation) at the surface of the steel and thus, improves the properties of surface of the steel, such as smoothness and evenness. However, when excess amounts of Cr are present, the toughness of the mother phase and the toughness at HAZ may be deteriorated. From this viewpoint, the content of Cr is preferably 0.7 % or less.

Ni is an element capable of improving the toughness of the mother steel. However, from the viewpoint of cost, the content of Ni is preferably 1.0 % or less.

Cu is an element capable of improving the strength of steel. However, when excess amounts of Cu are present, the hardenability of the steel may be excessively increased and thus the toughness of steel and the toughness at HAZ may be deteriorated. From this viewpoint, the content of Cu is preferably 1.0 % or less.

The structure of the alloy carbides and alloy carbonitrides and the mol fraction of precipitate of alloy carbides and alloy carbonitrides can be measured by observation and analysis using an electron microscope. As a simpler method, a software program for computing thermodynamic equilibrium can be used.

With respect to software usable in the present invention, for example, "Thermo-Calc" (manufactured by "Thermo Calc Software, USA)) can be employed for computing thermodynamic equilibrium. As a database, for example, "SSOL" can be also employed to carry out analysis. However, there is no limitation imposed on the software and database usable in the present invention, as long as the software and the database are dependable.

In the present invention, when the mol fraction of precipitate of alloy carbonitrides is computed, the total of two types of alloy carbides and alloy carbonitrides, i.e., the mol fraction of precipitate of alloy carbonitrides having a structure of Face Centered Cubic, which is on behalf of MCN type alloy carbonitrides and the mol fraction of precipitate of alloy carbides having a structure of Hexagonal Closed-Packed, which is on behalf of M₂C type alloy carbides, here, is defined as the mol fraction of precipitate of alloy carbides and alloy carbonitrides. Thus, the inventors compute both precipitate amounts of alloy carbides and alloy carbonitrides, and sum them up, and they apply the total precipitate amounts of the alloy carbides and the alloy carbonitrides as the mol fraction of precipitate. On this condition of calculation, the specific mol fraction of precipitate of alloy carbides and alloy carbonitrides are evaluated with respect to various kinds of elements and various temperatures.

It is necessary to add V, replacing partially Mo therewith, since Mo tends to form Mo-based alloy carbides which may be completely solid-soluted in steel at the temperature range of 600-650°C to fail to contribute to precipitation strengthening at such a high temperature. In the range of more than 0.20 % 0.35% of V content of the invention, the mechanical future at several temperatures, such as room temperature and high temperatures, are evaluated with respect to various kinds of alloy carbides and alloy carbonitrides and various mol fractions of precipitates thereof at various temperatures. This is done to investigate a suitable balance between the content of C and the content of N with particular focus on Mo and V included in alloy carbides and alloy carbonitrides.

It is preferred that the mol fractions of precipitates of alloy carbides and alloy carbonitrides are estimated by computing the thermodynamic equilibrium assuming that alloy carbides, which contain Mo mainly and in which V and/or Nb can also be solid-soluted, is "M₂C type alloy carbide", and alloy carbonitrides, which contain V and Nb mainly and in which Mo can be solid-soluted, is "MCN type alloy carbonitride". As the mol fractions of precipitates in the actual process using continuous cooling are slightly different from the mol fractions calculated above, it is preferable to make some corrections.

Mechanical properties at 600°C, especially proof stress of 0.2%, are preferred to attain excellent fire-resistance. Proof stress of 0.2% is preferably 157 MPa or more.

Changing the balance of elements, C and N used in the present invention, the properties of the shaped steel are evaluated at a range of 0-1.0 % of the mol fraction of precipitate of alloy carbides and alloy carbonitrides. It is found necessary that the mol fraction of precipitate of alloy carbides and alloy carbonitrides at 600°C is 0.3 % or more.

Further, in order to resolve a problem that the strength and yield ratio at room temperature is excessively increased, a suitable ratio of the mol fraction of precipitate of alloy carbides and alloy carbonitrides, i.e., the ratio of the mol fraction of precipitate of alloy carbides and alloy carbonitrides at 300 °C and that at 600 °C, and suitable mechanical properties at several high and room temperatures, are investigated. In order to simultaneously attain both a suppression of excessive increase of the strength at room temperature and an excellent fire-resistance, it is found necessary to meet the following condition i) impact strenght of Charpy impact test is 100 J or more at 0°C; and preferable to meet conditions: ii) tensile strength of the flange portion is 400 MPa or more; and iii) 0.2% proof stress at 600 °C is 157 MPa or more. Conditions i) and ii) are mainly for the properties at room temperature and condition iii) is mainly for the fire-resistance.

By changing the balance of elements, C and N used in the present invention in the presence of V replacing Mo partially therewith, the properties of the shaped steel are evaluated at range of 0-5.0 % of the mol fraction of precipitate of alloy carbides and alloy carbonitrides. It is found necessary that the ratio of the mol fraction of precipitate of alloy carbides and alloy carbonitrides at 300 °C and at 600 °C is 2.0 or less.

From the above investigation, precipitates of alloy carbides and alloy carbonitrides, which have excellent properties, can be newly obtained, as shown in Fig. 2 (a) and (b). In Fig.2(a) and (b), the amount of precipitate of alloy carbides of M₂C type containing partly V and Nb as a solid solution, alloy carbonitrides of MCN type containing mainly V, Nb and partly Mo as a solid solution, and the total of M₂C type alloy carbides and MCN type alloy carbonitrides are shown.

Fig.2 (a) shows the case where the content of V is 0.35%. The mol fraction of precipitate of alloy carbides and alloy carbonitrides at the temperature of 600 °C is 0.52%, which is within the range of the invention (0.3 or more). When the temperature is shifted from 600 °C to 300 °C, the mol fraction of precipitate of alloy carbides and alloy carbonitrides increases from about 0.52 % to about 0.54 %. The ratio of these is approximately 1.03, satisfying the condition of 2.0% or less of the invention.

Fig.2 (b) shows the case where the content of V is 0.22%. The mol fraction of precipitate of alloy carbides and alloy carbonitrides at the temperature of 600 °C is 0.52%, which is within the range of the invention (0.3 % or more). When the temperature is shifted from 600 °C to 300 °C, the mol fraction of precipitate of alloy carbides and alloy carbonitrides increases from about 0.52 % to about 0.59 %. The ratio between these is approximately 1.14, satisfying the condition of 2.0%

Thus, it is found that the composition design described above can simultaneously attain both a suppression of excessive increase of strength at room temperature and an excellent fire-resistance at 600°C.

Fig.3, on the other hand, shows the results where a conventional method is applied to a steel whose composition is within the range of the invention. As shown in Fig. 3, the mol fraction of precipitate of alloy carbides and alloy carbonitrides at 600 °C is within that of the invention (0.30% or more). However, when the temperature is shifted from 600 °C to 300 °C, the mol fraction of precipitate of alloy carbides and alloy carbonitrides increases drastically from about 0. 61 % to about 1.42 %. The ratio of the mol fraction of precipitate at 300°C and 600°C is 2.3, which is outside the range of the invention (2.0 or less). Fig.3 shows that the conventional method has a problem in that the strength at 300 °C is excessively high. It is noted that a conventional method is any method in which neither the mol fraction of precipitate of alloy carbides and alloy carbonitrides at 600°C is 0,3% more, nor the ratio of the mol fraction of precipitate of alloy carbides and alloy carbonitrides at 300°C to the mol fraction of precipitate of alloy carbides and alloy carbonitrides at 600°C is 2.0 or less.

The size of precipitates such as alloy carbides and alloy carbonitrides has an influence on the strength. In accordance with the desirable strength, it is preferred to make the precipitate fine-grained, for instance, to the size of 10-1000nm. It is preferred that solution treatment be conducted prior to hot rolling and precipitate be formed during cooling after hot rolling, or precipitate be formed by keeping the temperature of the steel at about 600 °C.

In the present invention, there is no specific limitation with respect to the ratio of the precipitate amounts between MCN type alloy carbonitrides having a stable less-temperature(only temperature range of 300°C to 600°C) -dependent precipitate amount and M₂C type alloy carbides having a temperature-dependent precipitate amount. It can be said, however, that the ratio, i.e., precipitate of MCN type alloy carbonitrides / precipitate of M₂C type alloy carbides (hereinafter referred to as the ratio of MCN/M₂C), is larger than that achieved by conventional methods. For example, a ratio of MCN/M₂C of 0.7 or more provides a significant effect at high temperatures, for example, 600°C. When the total amount of M₂C is reduced, however, the ratio of MCN/M₂C may not be a determining factor. In other words, the ratio of MCN/M₂C of 0.7 or more is not a required condition of the invention.

The reason for the limitation in the hot rolling process is as follows. First the casted steel, such as the slab, billet, bloom, near-net shape slab, ingot, etc., is reheated to a range between 1100 and 1300°C. The reason for the limitation of the temperature is to ensure a sufficient temperature to allow the casted steel to be processed in an austenite range and to sufficiently develop precipitation strengthening by making alloy carbides and alloy carbonitrides once a solid-solution in the process of hot rolling of the shaped steel.

After reheating, the casted steel is subjected to a hot rolling process. The hot rolling process basically includes a break-down process performed by groove rolling, intermediate rolling, and finishing rolling. The intermediate rolling process may be performed by any of a group of intermediate universal rolling machines including an edger rolling machine and a universal rolling machine, and the finishing rolling process may be performed by a universal rolling machine. The above-mentioned process also includes a rolling process using a skew roll for controlling the height of the web portion of the shaped steel.

In the break down process of the above rolling process, the casted steel is rolled in the width direction by a plurality of rolls, each roll has a groove of which bottom width is different to each other and the bottom part has a projected portion in the middle of the groove bottom. This is to ensure an appropriate flange width and web height.

In the intermediate rolling process, an appropriate flange width is obtained by an edger rolling machine and appropriate web thickness and flange thickness are obtained by an universal rolling machine. Furthermore in the finishing rolling process, shaped steel with predetermined size is formed while keeping the surface temperature of the flange portion, for instance, at 800°C or more.

The present invention can be preferably applied to a shaped steel of which the web thickness ranges from 9 mm to 40 mm, the flange thickness ranges from 12 mm to 60 mm, the web height is about 500 mm and the flange width ranges from 200 mm to 500 mm.

In the hot rolling process after the reheating, it is preferable that the shaped steel is water-cooled at least once to 700°C or less as measured at the surface of the flange portion and then rolled in the heat returning process.

As described above, the temperatures of the fillet and the flange portion are usually higher than that of the web portion due to the shape of shaped steel. In order to reduce the non-uniformity of the temperatures, the water-cooling of the flange portion and the rolling in the heat returning process are carried out at least once. Preferably this cyclic process of water-cooling and rolling can be repeatedly performed according to the size of shaped steel and the number of rolling passes.

In this invention, after finishing the hot rolling process, the shaped steel is either naturally cooled, or rapidly cooled, for instance, at least once, and then naturally cooled. In this cooling process the microstructure of the steel is fine-grained, which leads to improvements of strength at room temperatures, toughness and strength at high temperatures.

In the case where the rapid cooling is performed before natural cooling, the average cooling rate is preferably between 0.5 and 5.0°C/s so that the microstructure can be further fine-grained.

In the present invention, after performing the cooling process above-described, shaped steel excellent in fire-resistance having the following mechanical properties can be manufactured. That is, for example: mechanical properties where strength ratio defined by (0.2% proof stress at 600°C)/(yield strength at room temperature) is 50% or more, yield ratio at room temperature is 80% or less and Charpy impact absorption energy at 0°C is 100J or more; where the flange portion tensile strength at room temperature is 400 MPa class (grade), 0.2% proof stress at 600°C is 157 MPa or more and Charpy impact absorption energy at 0°C is 100J or more; and where the flange portion tensile strength at room temperature is 490 MPa class, 0.2% proof stress at 600°C is 217 MPa or more and Charpy impact absorption energy at 0°C is 100J or more.

### EXAMPLES

Examples of the present invention are described below. However conditions described in the examples are considered as illustrative only and the present invention is not restricted to these conditions. The invention can be applied in other various conditions without departing from the gist of the invention for accomplishing the object of the invention.

The steel blooms and billets used in these examples, having component (s) /composition (s) shown in Table 1 and the mol fractions of precipitates are predetermined through equilibrium calculation by the "Thermo-Calc" at 600 °C and 300°C, are melted in a steel converter and blooms and billets of about 240-300mm in thickness are cast in a continuous casting process. In Table 1, "tr" means "impossible to detect" or "unavoidable impurities".

The conditions of examples "a - g" of comparison steels, are outside the range of the invention. The conditions of components of example "a - c" are within that of the invention, but the mol fractions of precipitates of alloy carbides and alloy carbonitrides at 600 °C are not within the range of the invention (0.3 % and more). As for examples "d - g", each of the ratios of the mol fraction of the precipitate of alloy carbides and alloy carbonitrides at 300 °C to the mol fraction of the precipitate of alloy carbides and alloy carbonitrides at 600 °C, i.e., (the mol fraction at 300°C) / (the mol fraction at 600°C) are outside the range of the invention (2.0 and less).

In TABLE 1, the ratio of mol fraction of precipitate of alloy carbides and alloy carbonitrides at 300 °C to that at 600 °C shown in the rightmost column is not completely identical to the value calculated by each of the mol fraction of precipitate of alloy carbides and alloy carbonitrides at 300 °C and that at 600 °C. The difference is caused by number of significant digits, because each of the mol fraction of precipitate of alloy carbides and alloy carbonitrides are calculated to three decimal places, which is rounded off.

Each of the casted steel are reheated to 1100 - 1300°C and then subjected to the hot rolling process including a break-down process performed by a groove rolling process, an intermediate rolling process of a group of intermediate universal rolling machine including an edger rolling machine and a universal rolling machine, and a finishing rolling process performed by a universal rolling machine to form a H-shaped steel of predetermined size.

In the above hot rolling process, the web height of H-shaped steel is controlled by a rolling process using a skew roll.

H-shaped steel, of which the web thickness ranges from 9 mm to 40 mm, the flange thickness ranges from 12 mm to 60 mm, the web height is about 500 mm and the flange width ranges from 200 mm to 500 mm, are manufactured.

FIG. 1 shows a C-section of H-shaped steel, which is created by cutting the steel in a lateral direction (not longitudinal direction). The mechanical properties of the manufactured H-shaped steel are obtained by carrying out a variety of tests using a test piece (specimen). FIG.1 shows locations from where the test pieces (specimen) are taken. A first location is the center area of flange 2 in the thickness direction (1/2 t₂) and one-fourth (1/4 B) position of the total flange width (B) away from the end of flange 2 in the flange width direction. A second location is the center area of flange 2 in the thickness direction (1/2 t₂) and a half (1/2 B ) position of the total flange width (B) in the flange width direction (fillet part). A third location is the center area of web 3 in the thickness direction (1/2 t₁) and a half (1/2 H) position of the total web height (H) in the flange width direction. The mechanical properties at the above (1/4 B) position can represent the mechanical properties of the flange portion of H-shaped steel. However, the mechanical properties at the above three locations are measured and an average value of the mechanical properties of the three locations and a value of the mechanical property of the web portion (third location) are checked to confirm that excessive strengthening of mechanical properties with the web portion can be prevented. That is, a ratio of the value of the web portion to the average value of the three locations is calculated.

TABLE 2 illustrates the results of the above test, i.e., yield strength at room temperature, tensile strength at room temperature, yield ratio at room temperature, Charpy impact absorption energy at 0°C (3 points average value according to JIS, the specimen is JIS NO.4 (full size), with 2mm V-shape notch), 0.2% proof stress at 600°C according to JIS A2, and ratio of 0.2% proof stress at 600°C and yield strength at room temperature, for instance, according to JIS NO. 13A or 13B, depending upon the thickness of the shaped steel. As for the Charpy impact test, the data in TABLE 2 represents measured values of the fillet part (1/2 B) which has a lower value in the Charpy impact test than that of any other part in the section of the H-shaped steel. As for the 0.2% proof stress at 600°C, the data in TABLE 2 represent measured values of the (1/4 B) position in the flange portion. The value of the(1/4 B) position represents the strength of the H-shaped steel. There are two different classes (grades) of strength required to the steel. One is SN400 class, where the tensile strength at room temperature is 400 MPa and more, the other is SN490 class, where the tensile strength at room temperature is 490 MPa and more. As for SN400 class, examples whose strengths are approximately 400-520 MPa are shown. As for SN490 class, examples whose strengths are approximately 500-611 MPa are shown. In TABLE 2, the results are described according to the classes. Also, the ratio of the value of the mechanical property of the web portion to that of the average value of the three locations is calculated and listed therewith.

The steel of the invention satisfy such conditions as the components, and the mol fraction of precipitate of the alloy carbides and alloy carbonitrides. The mechanical properties of the steel of the invention attain the target properties both at high temperature (600 °C) and room temperature, such as yield strength, tensile strength, Charpy impact absorption energy at 0°C, particularly the strength ratio of the flange part of the steel is defined as (0.2 % proof strength at 600 °C)/(yield strength at room temperature) and yield ratio at room temperature.

The comparative examples, despite of having the same components as the steel of the present invention, do not satisfy at least one of the mechanical properties at room temperature and high temperature because they do not meet the requirements of mol fraction of precipitate of alloy carbides and alloy carbonitrides in the present invention.

Comparative steels "c, f, g" are insufficient in the Charpy impact absorption energy at 0°C in comparison with the steel of the present invention (100 J or more) . Comparative steels "a, b", belonging to class SN400, do not reach the target value of 0.2% proof strength at 600 °C, i.e., 157MPa and more. Comparative steels "d, e", belonging to class SN490, have a 0.2 % proof strength at 600 °C of 206, 212MPa respectively, which do not reach the target value of 217MPa and more. The strength ratios of comparative steels "d, e" do not reach the target value of 50% or more.

As previously mentioned, the present invention provides for shaped steel excellent in fire-resistance and having the desired strength at high temperature and mechanical properties at room temperature by forming alloy carbides and alloy carbonitrides mainly made of V and Mo under the proper balance of added amounts of V and Mo.

The shaped steel of the present invention is very useful as a construction material and has great industrial applicability.

All cited patents, publications, copending applications, and provisional applications referred to in this application are herein incorporated by reference.

The invention being thus described, it will be obvious that the same may be varied in many ways. Such variations are not to be regarded as a departure from the spirit and scope of the present invention, and all such modifications as would be obvious to one skilled in the art are intended to be included within the scope of the following claims.

**TABLE 1 High V content system**

| | | | | | | | | | | | | | | metal carbide and metal carbonitride precipitation by computing thermodynamic equilibrium | | |
|---|---|---|---|---|---|---|---|---|---|---|---|---|---|---|---|---|
| | NO | C | Si | Mn | Mo | V | N | Al | Ti | Nb | Cr | Ni | Cu | mol fraction at 600 °C (%) | mol fraction at 300 °C (room/ordinary temperature) (%) | ratio of mol fractions 300°C/600°C |
| H-shaped steel of the invention | 1 | 0.05 | 0.20 | 0.70 | 0.30 | 0.25 | 0.0043 | 0.010 | tr | tr | tr | tr | tr | 0.53 | 0.54 | 1.03 |
| | 2 | 0.05 | 0.20 | 0.60 | 0.15 | 0.35 | 0.0045 | 0.008 | tr | tr | tr | tr | tr | 0.54 | 0.55 | 1.03 |
| | 3 | 0.10 | 0.20 | 0.60 | 0.40 | 0.30 | 0.0045 | 0.008 | tr | tr | tr | tr | tr | 0.98 | 1.12 | 1.15 |
| | 4 | 0.07 | 0.10 | 1.05 | 0.30 | 0.35 | 0.0041 | 0.008 | tr | tr | tr | tr | tr | 0.73 | 0.75 | 1.03 |
| | 5 | 0.06 | 0.10 | 1.00 | 0.30 | 0.30 | 0.0073 | 0.008 | tr | tr | 0.2 | tr | tr | 0.65 | 0.67 | 1.03 |
| | 6 | 0.06 | 0.15 | 1.20 | 0.30 | 0.25 | 0.0070 | 0.010 | 0.012 | tr | tr | tr | tr | 0.64 | 0.73 | 1.14 |
| | 7 | 0.05 | 0.15 | 0.70 | 0.30 | 0.21 | 0.0041 | 0.010 | tr | tr | tr | tr | tr | 0.52 | 0.60 | 1.16 |
| | 8 | 0.10 | 0.20 | 0.60 | 0.40 | 0.25 | 0.0045 | 0.008 | tr | tr | tr | tr | tr | 0.89 | 1.16 | 1.31 |
| | 9 | 0.05 | 0.15 | 0.60 | 0.30 | 0.30 | 0.0047 | 0.008 | tr | tr | tr | 0.8 | 0.8 | 0.54 | 0.59 | 1.11 |
| | 10 | 0.12 | 0.10 | 1.01 | 0.40 | 0.35 | 0.0042 | 0.010 | tr | tr | tr | tr | tr | 1.11 | 1.35 | 1.21 |
| | 11 | 0.08 | 0.10 | 1.00 | 0.30 | 0.30 | 0.0073 | 0.008 | tr | tr | tr | tr | tr | 0.68 | 0.90 | 1.32 |
| | 12 | 0.05 | 0.10 | 1.05 | 0.20 | 0.21 | 0.0071 | 0.010 | tr | 0.03 | tr | tr | tr | 0.54 | 0.60 | 1.12 |
| H-shaped steel of comparison | a | 0.10 | 0.15 | 0.71 | 0.30 | tr | 0.0042 | 0.010 | tr | 0.02 | tr | tr | tr | 0.24 | 0.92 | 3.79 |
| | b | 0.10 | 0.15 | 0.72 | 0.30 | tr | 0.0042 | tr | tr | 0.04 | tr | tr | tr | 0.25 | 0.95 | 3.85 |
| | c | 0.10 | 0.15 | 0.75 | 0.30 | tr | 0.0044 | 0.010 | tr | 0.06 | tr | tr | tr | 0.27 | 1.06 | 3.87 |
| | d | 0.10 | 0.15 | 0.99 | 0.30 | 0.07 | 0.0073 | 0.008 | 0.010 | 0.04 | 0.2 | tr | tr | 0.41 | 1.38 | 3.37 |
| | e | 0.10 | 0.15 | 1.00 | 0.30 | 0,07 | 0.0074 | 0.008 | 0.010 | 0.06 | 0.2 | tr | tr | 0.34 | 1.36 | 3.97 |
| | f | 0.12 | 0.15 | 1.00 | 0.30 | 0.07 | 0.0071 | 0.001 | 0.005 | 0.04 | 0.2 | tr | tr | 0.41 | 1.65 | 3.97 |
| | g | 0.12 | 0.15 | 1.00 | 0.30 | 0.07 | 0.0073 | 0.001 | 0.010 | 0.06 | 0.2 | tr | tr | 0.45 | 1.63 | 3.61 |

**TABLE 2 high V content system**

| | | | | | | | mechanical poperties at room temperature | | | | | | mechanical property at high temperature | |
|---|---|---|---|---|---|---|---|---|---|---|---|---|---|---|
| | components | strength class | water cooling while rolling | rapid cooling (0.5-50°C /s) | thicknes- ratio of flange/we b (mm) | part of H-shaped steel | yield strength YP (MPa) | tensile strength TS (MPa) | yield ratio (%) | ratio of yield strength: web/ average | ratio of tensile strength web/ average | Charpy impact absorption energy at 0° C (J) *1 | 0.2% proof stress at 600° C PS(MPa) *2 | strength ratio: (0.2 % proof strength at 600 ° C)/ (yield strength at room temperature) (%) *3 |
| H-shaped steel of the invention | 1 | SN400 class | n/a | n/a | 20/35 | web portion | 334 | 426 | 78.4 | 104 | 1.03 | 389 | 182 | 54.5 |
| | | | | | | average | 322 | 415 | 77.6 | | | | | |
| | 2 | | applied | n/a | 14/26 | web portion | 338 | 427 | 79.2 | 1.03 | 1.02 | 346 | 185 | 54.7 |
| | | | | | | average | 327 | 418 | 78.2 | | | | | |
| | 3 | | applied | n/a | 13/21 | web portion | 349 | 441 | 79.1 | 1.04 | 1.02 | 264 | 191 | 54.7 |
| | | | | | | average | 335 | 432 | 77.5 | | | | | |
| | 4 | SN 490 class | applied | n/a | 14/26 | web portion | 417 | 542 | 76.9 | 1.03 | 1.02 | 280 | 229 | 54.9 |
| | | | | | | average | 406 | 533 | 76.2 | | | | | |
| | 5 | | applied | applied | 18/28 | web portion | 389 | 513 | 75.8 | 1.04 | 1.02 | 189 | 235 | 60.4 |
| | | | | | | average | 375 | 505 | 74.3 | | | | | |
| | 6 | | applied | n/a | 20/35 | web portion | 417 | 548 | 76.1 | 1.02 | 1.01 | 261 | 222 | 53.2 |
| | | | | | | average | 408 | 542 | 75.3 | | | | | |
| H-shaped steel of the invention | 7 | SN 400 class | n/a | n/a | 20/35 | web portion | 329 | 431 | 76.3 | 1.04 | 1.02 | 297 | 179 | 54.4 |
| | | | | | | average | 317 | 421 | 75.3 | | | | | |
| | 8 | | applied | n/a | 13/24 | web portion | 341 | 430 | 79.3 | 1.03 | 1.05 | 331 | 182 | 53.4 |
| | | | | | | average | 331 | 410 | 80.7 | | | | | |
| | 9 | SN 490 class | applied | applied | 13/21 | web portion | 384 | 512 | 75.0 | 1.05 | 1.04 | 184 | 220 | 57.3 |
| | | | | | | average | 367 | 494 | 74.3 | | | | | |
| | 10 | | applied | n/a | 13/24 | web portion | 398 | 544 | 73.2 | 1.05 | 1.03 | 201 | 234 | 58.8 |
| | | | | | | average | 378 | 527 | 71.7 | | | | | |
| | 11 | | applied | applied | 18/28 | web portion | 425 | 534 | 79.6 | 1.04 | 1.03 | 174 | 241 | 56.7 |
| | | | | | | average | 407 | 517 | 78.7 | | | | | |
| | 12 | | applied | n/a | 20/35 | web portion | 430 | 566 | 76.0 | 1.05 | 1.04 | 189 | 246 | 57.2 |
| | | | | | | average | 411 | 543 | 75.7 | | | | | |
| H-shaped steel of comparison | a | SN400 class | applied | n/a | 20/35 | web portion | 299 | 421 | 71.0 | 1.15 | 1.13 | 386 | 124 | 41.5 |
| | | | | | | average | 260 | 374 | 69.5 | | | | | |
| | b | | applied | n/a | 13/21 | web portion | 365 | 486 | 75.1 | 1.13 | 1.11 | 179 | 152 | 41.6 |
| | | | | | | average | 323 | 436 | 74.1 | | | | | |
| | c | | applied | n/a | 13/21 | web portion | 382 | 519 | 73.6 | 1.12 | 1.09 | 97 | 155 | 40.6 |
| | | | | | | average | 342 | 476 | 71.8 | | | | | |
| | d | SN490 class | applied | n/a | 14/26 | web portion | 415 | 575 | 72.2 | 1.1 | 1.09 | 197 | 206 | 49.6 |
| | | | | | | average | 377 | 529 | 71.3 | | | | | |
| | e | | applied | n/a | 14/26 | Web portion | 426 | 570 | 74.7 | 1.12 | 1.1 | 154 | 212 | 49.8 |
| | | | | | | average | 382 | 520 | 73.5 | | | | | |
| | f | | applied | n/a | 13/21 | web portion | 424 | 611 | 69.4 | 1.09 | 1.08 | 86 | 225 | 53.1 |
| | | | | | | average | 389 | 584 | 69.0 | | | | | |
| | g | | applied | n/a | 20/35 | web portion | 433 | 591 | 73.3 | 1.09 | 1.08 | 49 | 227 | 52.4 |
| | | | | | | average | 399 | 547 | 72.9 | | | | | |
| target properties : | | | | | | SN400 class | 235-355 | 400-510 | < 80 | | | 100 < | 157 < | 50 < |
| | | | | | | SN490 class | 325-445 | 490-610 | < 80 | | | 100 < | 217 < | 50 < |

| | | | | | | | | | | | | | | |
|---|---|---|---|---|---|---|---|---|---|---|---|---|---|---|
| **Bold number** : The bold numbers denote target property is unsatisfied. *1 test piece location for Charpy impact test : flange 1/2 B (fillet part) *2 test piece location for tensile test at high temperature: flange 1/4 B *3 yield strength at room temperature at web portion; 0.2 % proof strength at 600 ° C at flange 1/4 B | | | | | | | | | | | | | | |

## Claims

1. A shaped steel, comprising in mass percent (%):
C: 0.03-0.15;
Si: 0.05-0.50, Mn:0.4-2.0
Mo: 0.1- 0.6;
V: more than 0.20 to 0.35%; and
N: 0.002-0.012,
optionally Al ≤0.01, further optionally one or more of following elements in mass percent (%):
Ti : 0.005-0.020;
Nb ≤ 0.06 %;
Cr ≤ 0.7;
Ni ≤ 1.0; and
Cu ≤ 1.0
and the balance being iron and residual impurities, wherein
(x) a mol fraction of precipitate of alloy carbides and alloy carbonitrides at 600°C is 0.3 % or more, and
(y) a ratio of the mol fraction of precipitate of alloy carbides and alloy carbonitrides at 300°C to the mol fraction of precipitate of alloy carbides being M₂C type and alloy carbonitrides being MCN type at 600°C is 2.0 or less,
wherein a flange portion of the shaped steel has 50% or more of a ratio of strength, 80 % or less of yield ratio, and 100 J or more of impact strength of Charpy impact test at 0°C, wherein the ratio of strength = (proof stress of 0.2% at 600°C)/(yield strength at room temperature).

2. A method for producing a shaped steel according to claim 1 by hot rolling after reheating a casted steel, comprising steps of:
(a) reheating the casted steel to 1100 - 1300 °C;
(b) hot rolling the casted steel to form the shaped steel; and
(c) after terminating the hot rolling, naturally cooling or rapidly cooling then naturally cooling the shaped steel.

3. The method according to claim 2, wherein the step of hot rolling includes water-cooling the shaped steel at least once to 700°C or less as measured at the surface of a flange portion of the shaped steel and then rolling in the heat returning process.

4. The method according to claim 3, wherein the step of rapid cooling is performed at an average cooling rate of 0.5 to 5.0°C/s.

## Patentansprüche

1. Formstahl, umfassend in Gewichtsprozent (%):
C: 0,03 bis 0,15;
Si: 0,05 bis 0,50;
Mn: 0,4 bis 2,0;
Mo: 0,1 bis 0,6;
V: mehr als 0,20 bis 0,35%; und
N: 0,002 bis 0,012;
gegebenenfalls Al ≤ 0,01, weiter gegebenenfalls eines oder mehrere der folgenden Elemente in Gewichtsprozent (%):
Ti: 0,005 bis 0,020;
Nb ≤ 0,06%;
Cr ≤ 0,7;
Ni ≤ 1,0; und
Cu ≤ 1,0;
wobei es sich bei dem Rest um Eisen und vorhandene Verunreinigungen handelt, wobei
(x) die Molfraktion des Niederschlags aus Carbidlegierungen und Carbonitridlegierungen bei 600°C 0,3% oder mehr beträgt, und
(y) das Verhältnis der Molfraktion des Niederschlags aus Carbidlegierungen und Carbonitridlegierungen bei 300°C zur Molfraktion des Niederschlags aus Carbidlegierungen vom M₂C-Typ und Carbonitridlegierungen vom MCN-Typ bei 600°C 2,0 oder weniger beträgt,
wobei ein Flanschbereich des Formstahls ein Verhältnis der Festigkeit von 50% oder mehr, eine Streckgrenze von 80% oder weniger und eine Schlagzähigkeit beim Kerbschlagbiegeversuch nach Charpy bei 0°C von 100 J oder mehr aufweist, wobei das Verhältnis der Festigkeit = (Dehngrenze von 0,2% bei 600°C)/(Streckgrenze bei Raumtemperatur) ist.

2. Verfahren zur Herstellung eines Formstahls nach Anspruch 1 durch Warmwalzen nach dem Wiedererhitzen eines Gussstahls, umfassend die Schritte:
(a) Wiedererhitzen des Gussstahls auf 1100 bis 1300°C;
(b) Warmwalzen des Gussstahls, um den Formstahl zu bilden; und
(c) nach Beenden des Warmwalzens natürliches Abkühlen oder schnelles Abkühlen, gefolgt von natürlichem Abkühlen des Formstahls.

3. Verfahren nach Anspruch 2, wobei der Schritt des Warmwalzens das mindestens einmalige Abkühlen des Formstahls mit Wasser auf 700°C oder weniger, gemessen an der Oberfläche eines Flanschbereichs des Formstahls, und das anschließende Walzen während der erneuten Wärmezufuhr umfasst.

4. Verfahren nach Anspruch 3, wobei der Schritt des schnellen Abkühlens bei einer durchschnittlichen Abkühlgeschwindigkeit von 0,5 bis 5,0°C/s erfolgt.

## Revendications

1. Acier profilé, comprenant, en pourcentage de masse (%) :
C : 0,03-0,15 ;
Si : 0,05-0,50 ;
Mn : 0,4-2,0 ;
Mo : 0,1-0,6 ;
V : plus de 0,20 à 0,35 % ; et
N : 0,002-0,012 ;
en option Al ≤ 0,01,
en outre en option un ou plusieurs des éléments suivants, en pourcentage de masse (%) :
Ti : 0,005-0,020 ;
Nb≤0,06%;
Cr≤0,7;
Ni ≤1,0; et
Cu ≤ 1,0,
et le reste étant du fer et des impuretés résiduelles, dans lequel
(x) une fraction molaire de précipité de carbure allié et de carbonitrure allié à 600°C est 0,3 % ou plus, et
(y) un rapport de la fraction molaire de précipité de carbure allié et de carbonitrure allié à 300°C sur la fraction molaire de précipité de carbure allié étant du type M₂C et de carbonitrure allié étant du type MCN à 600°C est 2,0 ou moins,
dans lequel une partie en bride de l'acier profilé présente un rapport de résistance de 50 % ou plus, un rapport de rupture de 80 % ou moins, et une résistance aux impacts de 100 J ou plus dans un test d'impact de Charpy à 0°C, le rapport de résistance étant égal à
(contrainte d'épreuve de 0,2 % à 600° Celsius)/(résistance à la rupture à température ambiante).

2. Procédé pour produire un acier profilé selon la revendication 1, par laminage à chaud après réchauffement d'un acier coulé, comprenant les étapes consistant à :
(a) réchauffer l'acier coulé à 1100-1300°C ;
(b) laminer à chaud l'acier coulé pour former l'acier profilé ; et
(c) après avoir terminé le laminage à chaud, faire refroidir naturellement, ou faire refroidir rapidement puis refroidir naturellement: l'acier profilé.

3. Procédé selon la revendication 2, dans lequel l'étape de laminage à chaud inclut de refroidir à l'eau l'acier profilé au moins une fois jusqu'à 700°C ou moins, comme mesurer à la surface d'une portion de bride de l'acier profilé, puis de laminer dans le processus de retour de chaleur.

4. Procédé selon la revendication 3, dans lequel l'étape de refroidissement rapide est exécutée à une vitesse de refroidissement moyenne de 0,5 à 5,0°C/s.
